

# UNITED STATES PATENT OFFICE.

JOHN P. WOODS BECKMAN, OF PARNASSUS, PENNSYLVANIA.

## METHOD OF TREATING MICA.

No. 903,949.

Specification of Letters Patent.

Patented Nov. 17, 1908.

Application filed January 27, 1908. Serial No. 412,900.

*To all whom it may concern:*

Be it known that I, JOHN PIERSON Woods BECKMAN, a subject of the King of Sweden, residing at Parnassus, in the county of Westmoreland and State of Pennsylvania, have invented a new and useful Method of Treating Mica, of which the following is a full, clear, and exact description.

My invention has relation to a method of 10 treating mica for the purpose of rendering it flexible. It is well known that ordinary mica is very frangible, and that it can not be bent without cracking and breaking, which makes its use difficult or impossible 15 for many purposes for which it is otherwise specially adapted by reason of its insulating and other qualities.

The purpose of my invention is to provide 20 a simple and inexpensive method of treatment, whereby ordinary mica may be made flexible, so that it can be readily bent without injury.

In accordance with my invention, I take 25 sheets of mica of any desired thickness and immerse them in a bath of molten metal, in which I allow them to remain for a period depending somewhat upon the thickness of the sheets. I have secured excellent results with sheets of about one-thirtieth of an 30 inch in thickness, by allowing them to remain in a molten bath for a period of about one hour. While various metals may be used for the bath, I have found that aluminum is particularly well adapted for the 35 purpose. I have not been able to fully determine the exact nature of the effect which is produced upon the mica by this treatment, and whether a physical or a chemical change occurs, but inasmuch as the mica is rendered 40 flexible, by the treatment, to such an extent that sheets of a thickness of approximately one-thirtieth of an inch may be readily folded flat without breaking, it would appear that a substantial physical change occurs in the structure of the mica. This re-

sult is not effected by the deposition of the metal upon the surface of the mica, since, although when the sheets are removed from the bath, some of the metal may adhere thereto, yet this readily peels or flakes off, 50 and when it has been so removed, the remaining surfaces of the mica appear to show very little, if any, traces of the metal.

It will be understood that either the whole 55 or any portion of a mica sheet may be treated in accordance with my invention, only that portion which is treated being rendered flexible. The portion of a sheet which is not actually immersed in the bath, although it may be highly heated, does not become flexible.

By this simple and inexpensive method of treatment, I am enabled to produce mica which is very flexible and which can be used 65 for a variety of purposes, where difficulty is experienced in using the ordinary mica, by reason of its extreme frangibility.

I claim:

1. The method of treating mica to render it flexible, which consists in immersing it in 70 a molten bath, substantially as described.

2. The method of treating mica to render it flexible, which consists in immersing it in a bath of molten metal, substantially as described.

3. The method of treating mica to render it flexible, which consists in immersing it in a bath of molten aluminum, substantially as described.

4. The method of treating mica to render 80 it flexible, which consists in subjecting the mica in sheet form to the action of a bath of molten metal, substantially as described.

In testimony whereof, I have hereunto set my hand.

JOHN P. WOODS BECKMAN.

Witnesses:

H. M. CORWIN,  
GEO. H. PARMELEE.